

# UNITED STATES PATENT OFFICE.

JUNIUS D. EDWARDS, OF PITTSBURGH, FRANCIS C. FRARY, OF OAKMONT, AND HARRY V. CHURCHILL, OF PITTSBURGH, PENNSYLVANIA, ASSIGNEES TO ALUMINUM COMPANY OF AMERICA, OF PITTSBURGH, PENNSYLVANIA, A CORPORATION OF PENNSYLVANIA.

## MAKING CASTINGS OF ALUMINUM-SILICON ALLOYS.

1,410,461.

Specification of Letters Patent. Patented Mar. 21, 1922.

No Drawing.

Application filed November 27, 1920. Serial No. 426,796.

To all whom it may concern:

Be it known that we, JUNIUS D. EDWARDS, FRANCIS C. FRARY, and HARRY V. CHURCHILL, each a citizen of the United States of America, residing at, respectively, Pittsburgh, Oakmont, and Pittsburgh, in the county of Allegheny and State of Pennsylvania, have invented certain new and useful Improvements in Making Castings of Aluminum-Silicon Alloys, of which the following is a full, clear, and exact description.

This invention relates to aluminum alloys, particularly those containing silicon, and its chief object is to provide a method of making castings of such alloys which will improve the physical properties thereof, especially tensile strength and ductility. The invention is based on the discovery that the addition of sodium or potassium, or both, in metallic form, has an important effect upon the structure of the constituents, especially in the case of alloys containing silicon in substantial amounts.

Considerable variation is permissible in the proportions of the metals. In general, as the silicon content is increased the tensile strength of the alloy when cast in an ordinary sand mold is increased, up to a silicon content of about 10 per cent, but the elongation is decreased. For example, sand castings of an alloy containing ten parts of silicon to ninety parts of aluminum, in the form of cylindrical bars having a test section two inches long and a half inch in diameter, show an average tensile strength of about 20,000 pounds per square inch and an elongation of about 3 per cent, whereas similar castings of ordinary commercially pure aluminum have a tensile strength of about 12,000 pounds per square inch and an elongation of about 25 per cent. By means of the present invention it is possible not only to produce a substantial increase in the tensile strength of alloys containing silicon, but also to double and even treble the elongation.

In carrying out the invention in the preferred manner an alloy of aluminum and silicon is prepared, containing from 5 to 15 per cent silicon, approximately. This can be done, for example, by stirring metallic silicon in molten aluminum at a temperature

of about 750° to 800° C. To the alloy at this temperature the alkali metal or metals mentioned are added in metallic form and the melt stirred vigorously. Only a very small quantity of sodium or potassium is required, say about 0.1 per cent, but better results are obtained with sodium and potassium together, say about 0.05 per cent of each. For the best results the stirring should be rapid and the cast made promptly. The silicon content is preferably between 6 and 15 per cent, 8 to 13 per cent being usually the best. With the first mentioned percentage, round sand-cast bars having test sections two inches long and a half-inch in diameter showed a tensile strength of about 25,000 pounds per square inch and an elongation of from 12 to 14 per cent.

It is very desirable that the iron content be kept low, preferably less than 0.6 per cent, though in exceptional cases 1.5 per cent of iron may not be too high if ductility is not of great importance.

It has been observed that if the alloy after the addition of the alkali metal is allowed to stand in the molten state it is subject to a change which prevents the attainment of the best properties in the castings, and accordingly the cast should be made without undue delay after reaching proper pouring temperature, say 700° C. It is impossible to state definitely how long a time may elapse before casting and still realize the advantages of our invention, since that factor depends chiefly upon properties desired in the castings. With an increased amount of alkali metal a longer time may elapse without detriment to the product, but otherwise there is usually no material advantage but rather a disadvantage in employing more than the amount hereinbefore specified. It should not be understood that all the alkali metal added is to be found in the casting. A considerable portion of it is lost. The amount lost may, however, be reduced by the addition of the sodium and potassium in the form of an alloy with some other metal, for example zinc, in which case we have found that an addition of 0.02 per cent of the alkali metal accomplishes the same result as 0.1 per cent added directly.

In some cases the addition of a metal or

metals capable of forming solid solutions in aluminum, as for example copper and zinc, is advantageous. Thus the presence of copper up to about 0.5 per cent has a favorable effect upon the tensile strength. Copper to the amount of 0.3 per cent gives the maximum improvement in tensile strength without material decrease of ductility. However, the copper content can be increased up to 4 or 5 per cent with marked improvement in the physical properties of the alloy if the chill method of casting or the heat treatment described and claimed in the copending applications of Junius D. Edwards and Robert S. Archer, Serial No. 426,839, and Zay Jeffries and Robert S. Archer, Serial No. 435,024, be followed. In the first of these applications there is described a method which consists, broadly, in filling a suitable mold with the molten aluminum-silicon alloy and causing the latter to solidify rapidly, whereby precipitating silicon is caused to take the form of minute particles. The method described in the second of the above applications consists generally, in the case of aluminum-silicon alloys containing copper, in heating the alloy casting at a temperature slightly below the melting point of the eutectic until the silicon particles have been sufficiently altered and a sufficient amount of the inter-granular copper-rich constituent has been dissolved to materially improve the physical properties of the cast alloy. In general, when copper is present in considerable amount it is usually advisable to decrease the silicon content,—3 to 10 per cent silicon being generally suitable. The zinc may be added separately, or more or less of it (say about 1 per cent) may be introduced in the form of an alloy with the alkali metal, as herein-after described.

Microscopic examination shows that the addition of the above-mentioned alkali metals produces a change in the structure of the alloy, this change consisting in a marked reduction in the size of the silicon particles and a finer dispersion thereof. Thus in a sand-cast alloy containing silicon but without sodium or potassium the silicon is found in large plates or needles, whereas with the addition of either or both the metals named the silicon takes the form of very small particles, usually rounded or spherical, well distributed through the body of the eutectic. The addition of these alkali metals appears also to alter the composition of the eutectic alloy of the aluminum-silicon system. Without alkali metal the eutectic alloy contains about 11 to 12 per cent of silicon. Slowly solidified and untreated alloys containing less than that amount of silicon consist of eutectic plus excess aluminum, and those containing more silicon than the amount mentioned consist of eutectic plus

excess silicon. On the other hand, when the above-mentioned alkali metals are added there is a range of composition between 11 and 15 per cent silicon within which the alloy may behave as a eutectic, a hypo-eutectic, or a hyper-eutectic mixture. It has also been found that the change in the eutectic composition is usually accompanied by a lowering of the freezing point, in some cases as much as 12° C. below that of the normal aluminum-silicon eutectic.

In reduction of the particle size of the minor ingredient the effect of the addition of these alkali metals to aluminum-nickel alloys is similar to the effect in the case of aluminum-silicon alloys. In alloys containing copper the addition of sodium or potassium affects the primary grains and the cell size, making the primary grains smaller or larger according to the amount of alkali metal added, but in general making the cell size smaller.

In the foregoing description we have specified that the alkali metal is added in the metallic form, this mode of expression being employed for the purpose of excluding the use of the metals in the form of a salt. It is however not intended to exclude the addition of the alkali metal or metals in alloy with or in chemical combination with some other metal or metals; and as a matter of fact we have found that in some cases it is more convenient to add an alloy consisting of zinc 98 per cent and sodium 2 per cent, as explained more fully hereafter. The addition (in this manner) of alkali metal to the amount of 0.02 per cent simultaneously introduces zinc to the amount of about 1 per cent.

We have also discovered that cadmium and bismuth, to the amount of about 1 per cent or less, produce an effect similar to that obtained with sodium and potassium, but the use of cadmium and bismuth is not claimed specifically herein, as such use will form the subject of a later application.

As previously stated, there may be considerable loss attendant upon the introduction of the low melting and light alkali metal in pure form into the molten aluminum-silicon alloy. This loss can be reduced and further advantages secured by the use of an alloy of sodium or potassium, or both, with some heavy metal. For example, an alloy of sodium and zinc can be prepared, which contains about 2 per cent of sodium. This alloy is quite resistant to oxidation, and its alkali metal content does not necessitate taking any special precautions in handling it. Since this alloy has a relatively high melting point, it dissolves slowly in the molten aluminum-silicon alloy, and may be grasped in a pair of tongs and thoroughly incorporated into the alloy by stirring. Alloys of sodium or potassium, or both, with

other heavy metals can be used in place of the pure alkali metals in the manner described wherever the presence of the added amount of the alloying metal is not objectionable. The choice of the heavy metal to be alloyed with the alkali metal is determined in part by its effect on the properties of the resulting final alloy. The amount of alkali metal alloy required depends on its alkali metal content, and the efficiency of its utilization. As stated above, in the case of a sodium-zinc alloy, we have found that the use of enough to introduce .02 per cent sodium was sufficient to give satisfactory results.

The term "alkali metals" is commonly considered to include lithium, sodium, potassium, rubidium and caesium. Of these, only sodium and potassium are at all common or obtainable at a reasonable price and in commercial quantities. In many of its properties, lithium is more closely related to the metals of the alkaline earths than to sodium and potassium, and we find, as a matter of fact, that lithium does not produce the desired effect upon aluminum-silicon alloys. At the present time at least, rubidium and caesium are too rare to be commercially practicable for our purpose.

Castings made of aluminum-silicon alloys with addition of alkali metal as above described have shown themselves specially adapted for rolling and forging processes, both hot and cold. In general the fine structure produced by the alkali metal addition improves the quality of the alloys for any purpose where increased tensile strength and ductility are desired.

What we claim is—

1. In the art of making articles of aluminum alloy containing silicon in substantial amount, the improvement comprising adding to the molten alloy an alkali metal, and causing the alloy to solidify while sufficient alkali metal remains to favorably affect the structure of the alloy.

2. In the art of making articles of aluminum alloy containing silicon in substantial amount, the improvement comprising adding to the molten alloy metallic sodium, and causing the alloy to solidify while sufficient of the sodium remains to favorably affect the strength and ductility of the alloy.

3. In the art of making articles of aluminum alloy containing silicon in substantial amount, the improvement comprising adding to the molten alloy, alkali metal to the amount of 0.1 per cent approximately, and causing the alloy to solidify while sufficient alkali metal remains to favorably affect the structure of the alloy.

4. The method of making aluminum alloy castings of improved physical properties, comprising preparing an alloy of suitable composition, adding to the molten alloy a

relatively small amount of alkali metal, and casting the alloy while sufficient alkali metal remains to favorably affect the structure of the alloy.

5. The method of making aluminum alloy castings, comprising preparing an alloy of suitable composition containing a substantial amount of silicon, adding metallic sodium and potassium to the molten alloy, and casting the alloy while it retains enough of one or both metals to improve the physical properties of the alloy.

6. The method of making aluminum alloy castings, comprising preparing an alloy of suitable composition containing a substantial amount of silicon, adding to the molten alloy metallic sodium and potassium in the amount of not more than about 0.05 per cent. of each, approximately, and casting the alloy while it retains sufficient alkali metal to produce a substantial improvement in the physical properties of the alloy.

7. The method of making aluminum alloy castings, comprising preparing an alloy containing not less than about 3 nor more than about 15 per cent silicon, adding alkali metal to the molten alloy, and casting the alloy while it retains sufficient alkali metal to produce a substantial improvement in the physical properties of the alloy.

8. The method of making aluminum alloy castings, comprising preparing an alloy containing not less than about 3 per cent nor more than about 15 per cent silicon, adding metallic sodium to the molten alloy, and casting the alloy while it retains sufficient sodium to produce a substantial improvement in the physical properties of the alloy.

9. The method of making aluminum alloy castings, comprising preparing an alloy containing not less than about 3 per cent nor more than 15 per cent silicon, adding metallic sodium and potassium to the molten alloy, and casting the alloy while it retains sufficient alkali metal to produce a substantial improvement in the physical properties of the alloy.

10. The method of making aluminum alloy castings, comprising preparing an alloy containing 8 to 13 per cent silicon, approximately, adding alkali metal to the molten alloy, and casting the alloy while it retains sufficient alkali metal to produce a substantial improvement in the physical properties of the alloy.

11. The method of making aluminum alloy castings, comprising preparing an alloy containing about 8 to 13 per cent silicon, adding alkali metal to the amount of not more than about 0.1 per cent, and casting the alloy while it retains sufficient alkali metal to produce a substantial improvement in the physical properties of the alloy.

12. The method of making aluminum alloy castings, comprising preparing an alloy con-

taining about 8 to 13 per cent silicon, adding metallic sodium and potassium to the molten alloy, and casting the alloy while it retains sufficient alkali metal to produce a substantial improvement in the physical properties of the alloy.

13. The method of making aluminum alloy castings, comprising preparing an alloy containing about 8 to 13 per cent silicon, adding 10 to the molten alloy metallic sodium and potassium in the amount of not more than about 0.1 per cent, and casting the alloy while it retains sufficient alkali metal to produce a substantial improvement in the physical properties of the alloy.

14. The method of making aluminum alloy castings, comprising preparing an alloy containing copper and about 3 to 10 per cent silicon, adding to the molten alloy metallic 20 sodium and potassium in the amount of not more than about 0.1 per cent, and casting the alloy while it retains sufficient alkali metal to produce a substantial improvement in the physical properties of the alloy.

15. The method of making aluminum alloy castings, comprising preparing an alloy containing copper and about 3 to 10 per cent silicon, adding metallic sodium and potassium to the molten alloy, and casting the 30 alloy while it retains sufficient alkali metal to produce a substantial improvement in the physical properties of the alloy.

16. The method of making aluminum alloy castings, comprising preparing an alloy containing copper and about 3 to 10 per cent silicon, adding alkali metal to the amount of not more than about 0.1 per cent, and casting the alloy while it retains sufficient alkali metal to produce a substantial improvement in the physical properties of the alloy.

17. The method of making aluminum alloy castings, comprising preparing an alloy containing copper and not less than 45 about 3 per cent nor more than about 10 per cent silicon, adding metallic sodium to the molten alloy, and casting the alloy while it retains sufficient sodium to produce a substantial improvement in the physical properties of the alloy.

18. The method of making aluminum alloy castings comprising preparing an alloy containing copper and not less than about 3 nor more than about 10 per cent silicon, adding alkali metal to the molten 55 alloy, and casting the alloy while it retains sufficient alkali metal to produce a substantial improvement in the physical properties of the alloy.

19. The method of making aluminum alloy castings, comprising preparing an alloy of suitable composition containing copper and a substantial amount of silicon, adding to the molten alloy metallic sodium 65 and potassium in the amount of not more

than 0.05 per cent of each, approximately, and casting the alloy while it retains sufficient alkali metal to produce a substantial improvement in the physical properties of the alloy.

20. The method of making aluminum alloy castings, comprising preparing an alloy of suitable composition containing copper and a substantial amount of silicon, adding metallic sodium and potassium to 70 the molten alloy, and casting the alloy while it retains enough of one or both metals to improve the physical properties of the alloy.

21. The method of making aluminum alloy castings, comprising preparing an 80 alloy containing not less than about 3 nor more than about 15 per cent silicon, and copper in amount not more than about 0.5 per cent, adding alkali metal to the molten alloy, and casting the alloy while it retains sufficient alkali metal to produce a substantial improvement in the physical properties of the alloy.

22. The method of making aluminum alloy castings, comprising preparing an 90 alloy containing not less than about 3 nor more than about 15 per cent silicon and copper in amount not exceeding about 0.5 per cent, adding metallic sodium and potassium to the molten alloy, and casting the alloy 95 while it retains sufficient alkali metal to produce a substantial improvement in the physical properties of the alloy.

23. The method of making aluminum alloy castings, comprising preparing an 100 alloy containing 8 to 13 per cent silicon, proximity, and copper in amount not exceeding about 0.5 per cent, adding alkali metal to the molten alloy, and casting the alloy 105 while it retains sufficient alkali metal to produce a substantial improvement in the physical properties of the alloy.

24. The method of making aluminum alloy castings, comprising preparing an 110 alloy containing about 8 to 13 per cent silicon and copper in amount not exceeding about 0.5 per cent, adding to the molten alloy metallic sodium and potassium in the amount of not more than about 0.1 per cent, and casting the alloy while it retains sufficient alkali metal to produce a substantial improvement in the physical properties of the alloy.

25. The method of making aluminum alloy castings, comprising preparing an 120 alloy containing copper and zinc and about 8 per cent silicon, adding to the molten alloy metallic sodium and potassium in the amount of not more than about 0.1 per cent, and casting the alloy while it retains sufficient alkali metal to produce a substantial improvement in the physical properties of the alloy.

26. The method of making aluminum alloy castings, comprising preparing an 130

- alloy containing copper and zinc and not less than about 3 nor more than about 15 per cent silicon, adding metallic sodium and potassium to the molten alloy, and casting the alloy while it retains sufficient alkali metal to produce a substantial improvement in the physical properties of the alloy. 3. The method of making aluminum alloy castings, comprising preparing an alloy containing copper and zinc and not less than about 3 nor more than about 15 per cent silicon, adding alkali metal to the molten alloy, and casting the alloy while it retains sufficient alkali metal to produce a substantial improvement in the physical properties of the alloy. 27. The method of making aluminum alloy castings, comprising preparing an alloy containing copper and zinc and not less than about 3 nor more than about 15 per cent silicon, adding metallic sodium and potassium to the molten alloy, and casting the alloy while it retains sufficient alkali metal to produce a substantial improvement in the physical properties of the alloy. 28. The method of making aluminum alloy castings, comprising preparing an alloy of suitable composition containing copper and zinc and a substantial amount of silicon, adding metallic sodium and potassium to the molten alloy, and casting the alloy while it retains sufficient of one or both metals to improve the physical properties of the alloy. 29. The method of making aluminum alloy castings, comprising preparing an alloy containing zinc and about 8 to 13 per cent silicon, adding to the molten alloy metallic sodium and potassium in the amount of not more than about 0.1 per cent, and casting the alloy while it retains sufficient alkali metal to produce a substantial improvement in the physical properties of the alloy. 30. The method of making aluminum alloy castings, comprising preparing an alloy containing zinc and 8 to 13 per cent silicon, approximately, adding alkali metal to the molten alloy, and casting the alloy while it retains sufficient alkali metal to produce a substantial improvement in the physical properties of the alloy. 31. The method of making aluminum alloy castings, comprising preparing an alloy containing zinc and not less than about 3 nor more than about 15 per cent silicon, adding metallic sodium and potassium to the molten alloy, and casting the alloy while it retains sufficient alkali metal to produce a substantial improvement in the physical properties of the alloy. 32. The method of making aluminum alloy castings, comprising preparing an alloy containing zinc and not less than about 3 nor more than about 15 per cent silicon, adding alkali metal to the molten alloy, and casting the alloy while it retains sufficient alkali metal to produce a substantial improvement in the physical properties of the alloy. improvement in the physical properties of 60 the alloy. 33. The method of making aluminum alloy castings, comprising preparing an alloy of suitable composition containing a substantial amount of silicon and containing a 65 substantial amount of a metal capable of forming a solid solution in the aluminum, adding metallic sodium and potassium to the molten alloy, and casting the alloy while it retains enough of one or both metals to improve the physical properties of the alloy. 34. The method of making aluminum alloy castings, comprising preparing an alloy containing not less than about 3 nor more than about 15 per cent silicon, and 70 containing a metal capable of forming a solid solution in the aluminum, adding alkali metal to the molten alloy, and casting the alloy while it retains sufficient alkali metal to produce a substantial improvement in the 75 physical properties of the alloy. 35. The method of making aluminum alloy castings, comprising preparing an alloy containing about 8 to 13 per cent silicon, and containing a substantial amount of 80 metal capable of forming a solid solution in the aluminum, adding alkali metal to the amount of not more than about 0.1 per cent, and casting the alloy while it retains sufficient alkali metal to produce a substantial 85 improvement in the physical properties of the alloy. 36. The method of making aluminum alloy castings, comprising preparing an alloy containing about 8 to 13 per cent silicon and containing a substantial amount of 90 metal capable of forming a solid solution in the aluminum, adding to the molten alloy metallic sodium and potassium in the amount of not more than about 0.1 per cent, and casting the alloy while it retains sufficient alkali metal to produce a substantial 95 improvement in the physical properties of the alloy. 37. The method of making aluminum alloy castings, comprising preparing an alloy of suitable composition containing a substantial amount of silicon and of a metal capable of forming a solid solution in the 100 aluminum, adding alkali metal to the molten alloy, and casting the alloy while it retains enough alkali metal to improve the physical properties of the alloy. 105 In testimony whereof we hereunto affix our signatures.

JUNIUS D. EDWARDS.  
FRANCIS C. FRARY.  
HARRY V. CHURCHILL.